

# UNITED STATES PATENT OFFICE.

WILLIAM R. MOTT, OF LAKewood, OHIO, ASSIGNOR, BY MESNE ASSIGNMENTS, TO  
NATIONAL CARBON COMPANY, INC., A CORPORATION OF NEW YORK.

## ARC-LAMP ELECTRODE.

1,235,996.

Specification of Letters Patent.

Patented Aug. 7, 1917.

No Drawing.

Application filed September 25, 1914. Serial No. 863,463.

To all whom it may concern:

Be it known that I, WILLIAM R. MOTT, a citizen of the United States, residing at Lakewood, in the county of Cuyahoga and State of Ohio, have invented a certain new and useful Improvement in Arc-Lamp Electrodes, of which the following is a full, clear, and exact description.

My invention relates to arc light electrodes for producing a brilliant white light of high candle power, and is particularly adapted to photographic use.

The highest candle power in commercial arc lights has hitherto been obtained by the use of calcium fluorid as the main constituent, which produces a yellow flame. Yellow flame arcs are well adapted for lighting smoky or foggy places, on account of the great penetrating power of the yellow rays.

In certain cases, however, a pure white light is a desideratum, this being particularly true of photographic and photo engraving work. For general street lighting also, a white light is to be preferred.

In making flame electrodes for photographic and photo engraving work it has been customary to use rare-earth fluorids alone or in combination with other salts instead of using calcium fluorid. Calcium fluorid is considered to be the best all around flaming constituent that can be used in arc lamp electrodes, but the yellow character of its light has heretofore hindered its use in photographic lamps. My invention enables me to use calcium fluorid and thus obtain the high candle power incident thereto, while producing a snow white light.

Uranium in the electric arc probably gives more lines in the spectrum than any other known element, and the arc is exceptionally rich in the blue and violet rays, while it also contains a considerable number of ultra-violet rays. Uranium therefore has a unique distinction of giving 50% more photographic power when used in the arc than rare-earth fluorids, or titanium oxid, which have heretofore been considered the materials having the highest photographic values.

Uranium has a great propensity to form various chemical reactions with other substances when incorporated in the arc, and inasmuch as the candle power of the arc increases with the number of chemical com-

pounds that can be formed therein, uranium is a desirable material to be used in electrodes for this if for no other reason.

Uranium materials produce an arc having an intense blue center rich in actinic properties, and when it is mixed with calcium fluorid in making up an arc lamp electrode it fully blends with the yellow rays of the latter to produce an intense snow white light of extraordinary photographic power.

There are various uranium compounds that may be used to combine with calcium fluorid, such as the various oxids of uranium, uranates of calcium, strontium and other metals, metallic uranium, uranium carbide, uranium nitrid, uranium borate, uranium fluorid, uranium oxyfluorid and others.

Of the various compounds available I have found that the oxids of uranium and the uranates of calcium and strontium are the most efficient for the purpose mentioned. Uranium oxid or fluorid, when used alone in the arc, gives 50% more photographic power than any other material with which I am familiar.

Strontium uranate gives an arc with a red shell and an intense blue core so that the composite effect is a white light having 15 to 20% more photographic power than the rare-earth fluorids for instance, although most strontium compounds give hardly half the photographic power of such fluorids. This salt therefore, when used alone or in conjunction with other salts or materials capable of producing a white light, is very efficient as a flame constituent in white flamer.

The use of uranium salts and materials is not restricted to any definite amounts in proportion to the other materials in the electrode, but merely by way of example it may be stated that in cored electrodes for instance, the paste may consist of about 40% core black and 60% flaming material, which may consist entirely of uranium salts, oxids or other uranium material. When calcium fluorid is to be used in conjunction with uranium, the proper amount will be used to blend with the uranium rays to produce a snow white light.

Having described my invention, what I claim is:

1. An arc lamp electrode containing an

oxy-compound of uranium and a conducting body of carbon.

2. An arc lamp electrode containing calcium fluorid and a uranium material.

3. An arc lamp electrode containing calcium fluorid uranium material and a conducting body.

4. An arc lamp electrode containing cal-

cium fluorid an oxid of uranium and a conducting body.

In testimony whereof, I hereunto affix my signature.

WILLIAM R. MOTT.

Witnesses:

PHILIP P. BETHEA,  
H. G. GROVER.